

## UNITED STATES PATENT OFFICE

2,300,391

## LUBRICANT ADDITIVE

Meyer S. Agruss, Chicago, Hans Schindler, Evans-  
ton, and George W. Ayers, Jr., Chicago, Ill., as-  
signors to The Pure Oil Company, Chicago, Ill.,  
a corporation of Ohio

No Drawing. Application June 21, 1940,  
Serial No. 341,640

17 Claims. (Cl. 196—151)

This invention relates to lubricating oils and to processes for improving their properties and more particularly to the production of lubricating oils having green fluorescence and other desirable properties.

One of the objects of this invention is to provide petroleum lubricating oil possessing a green fluorescence from oils normally deficient in that property.

Another object is to provide a method of preparing a green bloom agent.

A further object is to provide a green bloom agent useful in imparting a green fluorescence to oils normally deficient in that property.

A still further object is to provide a method of preparing lubricating compositions possessing a green fluorescence from lubricants normally deficient in that property.

Other objects and advantages will be apparent from the following detailed description.

Certain lubricating oils such as those derived from naphthenic and mixed base crudes, while possessing good lubricating characteristics, are, nevertheless, deficient in the property of bloom. Pennsylvania lubricating oils are reddish brown by transmitted light and green by reflected light, thereby possessing what is known as a green bloom or fluorescence. The trade acceptance of oils having a green bloom is superior to that of oils which do not possess such a bloom and it is therefore desirable in certain cases to impart a green bloom to such lubricating oils which are deficient in this property.

It has been discovered that a very satisfactory green bloom imparting material may be prepared by condensing petroleum resins with halogenated, preferably chlorinated, hydrocarbons, particularly those hydrocarbons of the paraffin series. Condensation may be effected by any of the well known condensing agents such as metallic halides, especially aluminum chloride. A convenient and economical source of suitable paraffin hydrocarbons is commercial paraffin wax or petrolatum. These products are obtained in the course of conventional refining methods as applied to the manufacture of lubricating oils.

Petroleum resins preferable for the condensation reaction are those resins obtained from spent or partially spent adsorbents such as fuller's earth which have been used in decolorizing operations on petroleum oils such as neutral oils, bright stocks and cylinder stocks. Such resins may be conveniently obtained by extracting the spent adsorbents with chloroform or a mixture of benzol and alcohol or similar solvents. In

order to reduce the amount of oil in the resins the spent adsorbent is preferably washed with petroleum naphtha prior to the extraction with benzol and alcohol or chloroform. The resin may be readily separated from the solvent-resin solution by distillation and is obtained as a dark brown viscous fluid. If the petroleum oil which is decolorized by contact with the adsorbent contains excessive asphaltic material, it may be desirable to separate at least a portion of this asphaltic material prior to contact with the decolorizing adsorbent. This may be readily accomplished by any of several well known de-asphaltizing methods, for example, by the use of propane.

Suitable resins may also be obtained in the course of refining gasoline and similar light distillates produced by cracking hydrocarbon oils, particularly in the cracking of hydrocarbon oils at more elevated conversion temperatures, such as approximately 1000° F. or higher and in the refining of gasoline or similar boiling range material produced by conversion or polymerization of hydrocarbon gases. The gasoline or similar distillate is contacted with polymerizing catalyst such as fuller's earth or similar adsorptive clay at elevated temperature in order to selectively polymerize gum-forming and color-imparting constituents contained therein to resins. These gum-forming or color-imparting constituents are usually diolefins which readily polymerize and oxidize upon exposure to air and/or light.

In the well known Gray process cracked gasoline vapors are passed through a tower containing a bed of adsorbent clay at temperatures ranging from approximately 200—400° F. and the resulting resin-containing liquid withdrawn from the bottom of the tower.

In another method of refining cracked distillates adsorbent clay is either mixed with the distillate under sufficient pressure to maintain the distillate in substantially liquid phase and the mixture heated at temperatures of approximately 400—600° F. for a sufficient period of time to bring about the desired polymerization of gum-forming or color-imparting bodies; or the distillate is passed through a chamber packed with adsorbent clay under high pressure conditions and at elevated temperatures and the desired polymerization effected, the desirable resins being separable from the polymer distillate by fractional distillation.

Suitable resins of a similar nature may also be obtained from the treatment of cracked distillates with selective polymerizing agent such as

dilute sulfuric acid or cold concentrated sulfuric acid.

The methods hereinabove set forth for the selective polymerization of gum-forming and color-imparting bodies in cracked distillates are well known in the art and produce resins suitable for use in this invention. While the polymerized fractions produced by any of the aforementioned methods may contain a sufficiently high proportion of resins to be directly used in this invention, it is frequently desirable to concentrate the resins by fractional distillation of the polymerized fractions, the resins being obtained as the less volatile portion of the polymers.

As an example of the preparation of green bloom agents in accordance with this invention, petrolatum of approximately 140° F. melting point was chlorinated to a chlorine content of approximately 10%. In general it is preferred to have approximately 10% to 25% chlorine by weight. Temperature during chlorination was preferably controlled so as to be not substantially in excess of 300° F. The chlorinated product was mixed in the proportion of two parts by weight of chlorinated product to three parts by weight of hydrocarbon resin obtained from partially spent decolorizing clay which had been used to decolorize Pennsylvania cylinder stock. This resin was obtained by first washing the spent clay with naphtha to remove any oil that may have been present and then extracting the naphtha-washed clay with chloroform. The chloroform was distilled from the resin-chloroform solution and the resin obtained as a dark brown, sticky fluid of approximately 1.02 specific gravity and about 590 seconds Saybolt Universal viscosity at 210° F. The chemical condensation of the chlorinated petrolatum and resin was effected by adding 10% by weight based on the resin, of anhydrous aluminum chloride to the mixture as a condensation catalyst and gradually heating to a temperature of approximately 200° F. to 220° F. This temperature was maintained until the reaction was complete, which in this case was about forty-five minutes. The completeness of the reaction was readily determined by the cessation of the evolution of hydrogen chloride gas. This produces a reaction product that is substantially free of combined chlorine. The temperature at which the condensation reaction may be carried out may vary considerably, but preferably should not exceed 300° F. Ordinary atmospheric pressure is satisfactory. The condensation reaction was carried out under conditions of constant agitation in carbon tetrachloride which functioned solely as a solvent to diminish the viscosity of the mixture. When the reaction was complete, reaction products insoluble in the carbon tetrachloride solution were removed by water washing. The soluble reaction product was readily separated from carbon tetrachloride by fractional distillation. This reaction product contained only a very small amount of chlorine which was present as an impurity due to incomplete removal in water washing.

The effect of the addition of additive prepared as set forth in the preceding paragraph, on the bloom of a Gulf Coast lubricating oil was determined. The oil prior to mixture with the additive possessed a definitely blue bloom. After addition of 1.0% of additive the oil possessed a green bloom. It is apparent that the shade of bloom imparted to oils may be varied with the amount of additive used. The amount of additive

generally used is of the order of 0.1% to 10%, although there is no reason why greater or lesser amounts cannot be used since the additive is itself a good lubricant.

5 While material prepared in accordance with this invention is extremely useful as a green bloom imparting agent, the material is also useful as a wax crystal modifying agent in the dewaxing of wax-bearing lubricating oils and in depressing the pour point of mineral lubricating oils when used in the amounts above indicated. It is also possible to simultaneously impart green bloom and depress the pour point of certain oils, such as some wax-bearing Mid-Continent lubricating oils which are deficient in green bloom and of relatively high pour test.

10 The amount of aluminum chloride used may vary between wide limits, but in general it is preferred to use approximately 2% to 10% by weight of aluminum chloride based on the resin.

15 The proportion of hydrocarbon resin to chlorinated petrolatum which may be used may be varied between rather wide limits. In general it has been found that most satisfactory results were obtained by using approximately three parts of hydrocarbon resin to two parts of chlorinated petrolatum.

20 The foregoing specific description is given by way of illustration only and not by way of limitation, the invention being limited only as indicated by the appended claims.

25 What is claimed is:

1. A lubricant possessing a green fluorescence comprising lubricating oil normally deficient in green fluorescence and a minor portion of petroleum resin-halogenated hydrocarbon condensation product.

30 2. A lubricant in accordance with claim 1 where the resin is obtained from partially spent decolorizing adsorbent used in the decolorization of hydrocarbon oils.

35 3. A lubricant in accordance with claim 1 where the petroleum resin is obtained from selective polymerization of diolefin-containing hydrocarbon distillates.

40 4. A lubricant in accordance with claim 1 where the halogen is chlorine.

45 5. A lubricant in accordance with claim 1 where the proportion of hydrocarbon resin to halogenated hydrocarbon is approximately 3 to 2.

50 6. A lubricant possessing a green fluorescence comprising lubricating oil normally deficient in green fluorescence and a minor portion of petroleum resin-chlorinated paraffinic hydrocarbon condensation product.

55 7. A lubricant in accordance with claim 6 where the paraffinic hydrocarbon is petrolatum.

60 8. A lubricant in accordance with claim 6 which contains 0.1% to 10% of condensation product.

65 9. A lubricant in accordance with claim 6 where the chlorinated hydrocarbon contains approximately 10% to 25% chlorine.

70 10. Method of producing a green bloom lubricating oil which comprises adding to petroleum lubricating oil normally deficient in green bloom, condensation product of halogenated hydrocarbon and petroleum resin.

75 11. Method in accordance with claim 10 where the halogenated hydrocarbon is chlorinated paraffinic hydrocarbon.

12. Method in accordance with claim 10 where the petroleum resin is obtained from partially spent decolorizing adsorbent used in the decolorization of hydrocarbon oils.

13. Method in accordance with claim 10 where the petroleum resin is obtained from selective polymerization of diolefin-containing hydrocarbon distillate.

14. Method of preparing a green bloom imparting agent comprising chemically reacting halogen with hydrocarbon, mixing the halogenated hydrocarbon with petroleum resin and a condensation agent, heating the mixture to elevated temperature and maintaining the temperature for a sufficient time to effect condensation of the halogenated hydrocarbon and petroleum resin and separating the condensation product from the reaction mixture.

15. Method in accordance with claim 14 where 15

the halogen is chlorine and the hydrocarbon is paraffinic hydrocarbon.

16. Method in accordance with claim 14 where the halogen is chlorine, the chlorine comprises 10% to 25% by weight of hydrocarbon and the ratio of hydrocarbon resin to chlorinated hydrocarbon is approximately 3 to 2.

17. Method of imparting green bloom and reducing the pour test of wax-bearing lubricating oil normally deficient in green bloom which comprises adding to said oil condensation product of halogenated hydrocarbon and petroleum resin.

MEYER S. AGRUSS.

HANS SCHINDLER.

GEORGE W. AYERS, JR.